

Aug. 30, 1927.

1,640,795

J. S. MILLER, JR

WATERPROOF FABRIC AND ITS MANUFACTURE

Filed April 29, 1925

***FIG. I.***



***FIG. II.***



WITNESSES

Alfred E. Schinger  
Thomas W. Kerr, Jr.

INVENTOR:

John Strother Miller, Jr.  
BY Tracy & Paul  
ATTORNEYS.

Patented Aug. 30, 1927.

1,640,795

# UNITED STATES PATENT OFFICE.

JOHN STROTHER MILLER, JR., OF RAHWAY, NEW JERSEY, ASSIGNOR TO THE BARBER ASPHALT COMPANY, OF PHILADELPHIA, PENNSYLVANIA, A CORPORATION OF WEST VIRGINIA.

## WATERPROOF FABRIC AND ITS MANUFACTURE.

Application filed April 29, 1925. Serial No. 26,603.

My invention relates to waterproof fabric and the like, and its manufacture. I aim to provide a material whose appearance and other properties adapt it for use as a substitute for leather, as well as for various other purposes. I also aim to reduce the cost of manufacture of such a product to the minimum consistent with satisfactory quality.

How these and other advantages can be realized through my invention will appear from the description hereinafter of one mode of manufacturing such a material, especially when considered in connection with the following explanation of present practice in the manufacture of artificial leather.

At the present time, artificial leather commonly consists of a fabric base (either a textile fabric or a felted one) coated with a film of "dope" mixture adapted to simulate leather in appearance and "feel". Such a dope usually comprises a soluble cotton or pyroxylin varnish, with an admixture of castor oil or other suitable oil to render the dried film flexible, and with suitable dyes or pigments to give the product the desired color. In order to give the product the necessary thickness or body, either the fabric base or the coating of dope (or both) must be relatively thick. This is practically disadvantageous, however, particularly owing to the relatively high cost entailed by the use of so much dope or of such heavy fabric.

I have discovered that such drawbacks of present practice can be overcome by employing a bitumen-coated fabric in such artificial leather or the like, instead of a plain fabric, as heretofore used; so that only a relatively thin coating or film of leather-simulative varnish or dope will be required,—or even, for some purposes, none at all. Preferably, the fabric base is impregnated with bitumen before being coated therewith. If both sides of the fabric base be coated with bitumen (even though only one is to be finished and exposed in use), the base will be protected from moisture, and the life of the product prolonged. On the side (or sides) of the product that is exposed in service, the dope coating protects the bitumen from too easy abrasion or indentation; while the asphalt coating (coatings) give the necessary thickness or body with much less dope than here-

tofore required, and with thinner (though not necessarily weaker) fabric.

In the drawings,

Fig. I is a perspective view of a piece of material embodying my present invention, with various outer layers removed over certain areas to show its construction.

Fig. II is a diagrammatic side view illustrating the manufacture of such a product.

The piece of artificial leather shown in Fig. I comprises a base 5 of any suitable fabric, here indicated as of textile character, such as a stout muslin. Preferably, this base 5 is impregnated and saturated with bitumen, as hereinafter described. In the present instance, the base 5 has a coat of bitumen 6 on both sides, but is finished with a surface film or coat 7 of dope or varnish on one side only.

Fig. II illustrates diagrammatically one method of manufacturing such a product. As here shown, a web of the unimpregnated base fabric 5 is drawn from a supply roll 11 by and between a pair of feed rolls 12, 12. From the rollers 12, 12, the fabric 5 passes down around a guide roll 13 immersed in a heated bath 14 of suitable molten bitumen, with which the fabric is thus impregnated and preferably saturated. The impregnated fabric is drawn from the bath 14 by and between a pair of rolls 15, 15. Molten bitumen is delivered by a supply pipe 16 on top of the impregnated fabric in front of the upper roll 15. This upper roll 15 spreads the bitumen evenly over the fabric 5 and the excess falls from the edges of the fabric into a trough 17. The lower roll 15, dipping into the bitumen in this trough or pan 17, applies the bitumen to the lower side of the fabric. Thus the fabric is thoroughly impregnated and coated with bitumen,—in the present instance, on both sides. Leaving the rolls 15, the coated fabric cools on its way to a pair of finishing and feed rolls 20, 20, which smooth out any inequalities and bring the coated product to a uniform thickness. If desired, one or both of the rolls 20, 20 may be suitably surfaced to impart to the bitumen coating 6 of the fabric 5 a configuration simulative of a natural or an artificial leather finish or decoration, such as a grained, pebbled, or veined surface, or any desired embossed or depressed ornamental design. From the rolls 20, 20, the bituminous coated product passes over a dope or

varnish spray 21 (above a drip pan or bath 22), thus receiving a thin surface coat or film 7 of the dope or varnish. This film 7 dries and hardens on the way to the roll 23, 5 on which the finished product is finally wound-up.

For impregnating the base fabric 5 may be used any bituminous material of such properties that it will neither soften nor 10 crack under the range of temperature to which it may be subjected in service: e. g., a composition of fluxed natural or artificial asphalts. For stiffer types of products, where pliability is not a factor, very hard 15 saturations may be used; but when pliability is desired, softer saturations must be employed,—such as are now used for impregnating the paper felt base of prepared roofing. For the bituminous coating 6 may 20 be used a bitumen of similar properties, except that it need not be so fluid or soft, since it does not have to soak, penetrate, and saturate the fibres of the base. A composition of blown or oxidized asphalt may be 25 used, either with or without softening oils (fluxed or unfluxed). The composition may and must be harder for stiffer or less pliable products, and softer for more pliable ones. In either case, it must be of such melting 30 point as to prevent undue softening under atmospheric temperatures. This minimum melting point may be as low as 175° F., Ring and Ball method.

The dope or varnish employed for the 35 surface finish may be such as now used for the manufacture of artificial leathers, as above described, but preferably somewhat thinner in consistency, in order to give a correspondingly thinner film or coating on 40 the bitumen-coated base. For example, a pyroxylin or soluble cotton varnish with an addition of castor oil to render it flexible, and of dye or pigment to give the desired

color, answers the purpose very satisfactorily. Such a coat 7 protects the finish, 45 configuration, or design imprinted in the bitumen by the rolls 20, 20.

Having thus described my invention, I claim:

1. A waterproof fabric of the character 50 described, comprising a bitumen-saturated coated textile fabric varnished with a flexible leather-simulative varnish.

2. A waterproof fabric of the character 55 described, comprising a bitumen-impregnated-coated textile fabric base, varnished with a flexible protective leather-simulative varnish.

3. A waterproof fabric of the character 60 described, comprising a textile fabric base saturated and coated on one face with asphalt, and varnished on said coated face with a flexible colored pyroxylin varnish.

4. A waterproof fabric of the character 65 described, comprising an asphalt-saturated-coated textile fabric base embossed with a leather-simulative design on the coated face and varnished with a flexible protective leather-simulative varnish.

5. The process of manufacturing a water- 70 proof fabric of the character described which comprises impregnating and coating on one face a textile fabric base with bitumen, and varnishing the coated face with a flexible leather-simulative varnish.

6. The process of manufacturing a water- 75 proof fabric of the character described which comprises imprinting a bitumen-saturated-coated textile fabric base with a leather-simulative design, and varnishing the coated face with a flexible protective leather-simulative varnish.

In testimony whereof, I have hereunto signed my name at Maurer, New Jersey, this 21st day of April, 1925.

JOHN STROTHER MILLER, JR.